

Patented Aug. 12, 1947

2,425,393

# UNITED STATES PATENT OFFICE

2,425,393

## HYDROXYLATED POLYAMIDE TEXTILE LUBRICANTS

Edwin A. Robinson, Chatham, and Maurice J. Kelley, Newark, N. J., assignors to Nopco Chemical Company, Harrison, N. J., a corporation of New Jersey

No Drawing. Application June 23, 1943,  
Serial No. 491,970

11 Claims. (Cl. 260—404.5)

1

This invention relates to textile lubricants and softeners, and more particularly to textile lubricants and softeners comprising mixed fatty polyamides. This application is a continuation-in-part of our copending application Serial No. 274,808, filed May 20, 1939, now Patent No. 2,345,632.

It has been proposed to use higher fatty amides such as oleic acid amide, oleic acid methyl amide and oleic acid ethylene diamide as softeners and lubricants for textile materials. Such amides are ordinarily prepared by reacting a fatty acid or fatty ester with a mono- or polyamide. The reaction of monoamines with higher fatty acids or fatty esters yields products which are not readily dispersible in water and since these products contain no residual amino group they cannot be solubilized to any substantial extent by treatment with acids. Hence, these products cannot be advantageously applied to textile material. It has been proposed, therefore, to react polyamines with higher fatty acids or fatty esters to produce amides having free amino groups capable of reacting with weak acids so as to solubilize the products and render them readily dispersible or soluble in water. However, the monoamides formed by such polyamines by reaction thereof with higher fatty acids or fatty esters cause yellowing of textile material upon application thereto and hence are highly unsuitable for use as textile lubricants and softeners. On the other hand, polyamides formed by the reaction of higher fatty acids or fatty esters with polyamines are much less desirable as softeners and lubricants than the corresponding monoamides because of their relatively poor softening and lubricating properties.

It has also been proposed to prepare textile lubricants and softeners by reacting unsymmetrical dialkyl ethylene diamines with higher fatty acids such as oleic acid. Such unsymmetrical dialkyl amines are, however, relatively expensive and difficult to obtain and hence, while amides thereof have been used to some extent as textile lubricants and softeners, there is a great demand in the textile industry for cheaper products which may be used in place of these amides.

It is an object of this invention to provide inexpensive and highly effective textile lubricants and softeners.

2

It is a further object of this invention to provide a process for the preparation of textile lubricants and softeners from polyamines.

The foregoing objects are secured and the disadvantageous features of the compositions produced in accordance with the prior art are overcome in polyamides having the general formula:



or preferably the more specific formula:



wherein:



20 represents a fatty acyl radicle containing from 8 to 22 carbon atoms;



25 represents a fatty acyl radicle containing from 1 to 5 carbon atoms; Z represents an aliphatic linking chain having an unsatisfied valence at both ends thereof, such as aliphatic hydrocarbon radicles; aliphatic hydrocarbon radicles having

30 a hydrogen atom replaced by a hydroxyl group; and aliphatic hydrocarbon radicles and aliphatic hydrocarbon radicles having a hydrogen atom replaced by a hydroxyl group, which radicles may be interrupted by one or more ether, imino, neutralized imino, amido or keto groups; R<sub>3</sub> in each occurrence, and independently of every other occurrence, represents a hydrogen, an alkyl group or an alkylol group, with the proviso that at least one of the R<sub>3</sub> substituents must be an alkylol group, or alternatively, in the case of Formula

35 1 the radicle Z may satisfy the proviso by containing a hydroxyl group; R<sub>4</sub> in each occurrence, and independently of every other occurrence, represents a hydrogen atom or an alkyl radicle; and

40 n represents a small whole number.

Such hydroxylated polyamides may be applied to textile materials, and when so applied impart thereto excellent softness, drape and pliability without causing yellowing of the material. The

45 50 polyamides of our invention may be prepared in

a simple and inexpensive manner by reacting a readily available hydroxylated polyamine having the general formula:



or preferably an ethylene polyamine having the more specific formula:



under the notation of formulae (1) and (2) supra, with a fatty acid containing from 8 to 22 carbon atoms, or an ester or acid halide thereof, and with a short chain fatty acid containing from 2 to 5 carbon atoms. Under the general formulae (1) and (2) it is possible for the polyamides to contain one or more secondary amino groups, in which case they may be converted to salts by means of weak acids to enhance the solubility thereof. We have found, however, that the presence of substantially more than one secondary amino group in the hydroxylated polyamides of our invention tends to cause yellowing of any textile material to which the polyamides are applied; hence, if hydroxylated polyamines containing more than 3 nitrogen atoms, e. g., ethanol triethylene tetramine, are employed to prepare the products of our invention, preferably, sufficient amounts of the short chain fatty acids are employed so as to acylate at least all but one of the secondary amino groups.

The products of our invention are preferably prepared by reacting a hydroxylated polyamine with a higher fatty acid containing from 8 to 22 carbon atoms, preferably 12 to 18 carbon atoms, or an ester thereof so as to form a monoamide, and then reacting the monoamide with suitable amounts of an acid containing from 2 to 5 carbon atoms. However, when employing diamines or triamines in the practice of our invention, the preparation of the amides may be carried out by first reacting the polyamine with the short chain acid and then treating the product with the long chain fatty acid. Any hydroxylated polyamine may be used in the practice of our invention; thus, for example, hydroxylated polyamines such as ethanol ethylene diamine, ethanol diethylene triamine, ethanol propylene diamine, symmetrical diethanol ethylene diamine, 1 amino 3 methylamino isopropanol, N ethyl N' ethanol ethylene diamine, isopropanol ethylene diamine, 1 amino 2 ethyl 3 ethanol amino isopropanol, 1-aminodimethyl 5 methylaminodimethyl n-pentanol-3, 1,3 diamino isopropanol, etc., all coming within the formulae (3) and (4), supra, may be employed. Products of those amines containing 3 or more nitrogen atoms may be converted to salts to enhance the solubility thereof; however, the hydroxyl and short chain acyloxy groups themselves impart a considerable degree of solubility and assist dispersion; accordingly, products prepared from ethanol ethylene diamine have been found highly satisfactory without conversion to the salt and for this reason, as well as on account of its cheapness, ethanol ethylene diamine is a highly preferred starting material for the synthesis of compositions according to this invention.

The long chain fatty acid compound reacted with the polyamine in accordance with our invention may be any of the fatty acids containing from 8 to 22 carbon atoms, preferably from 12 to 18 carbon atoms, or the esters thereof; the

following higher fatty acids may be mentioned by way of examples: caprylic acid, nonyl acid, capric acid, undecylic acid, lauric acid, myristic acid, palmitic acid, stearic acid, behenic acid, oleic acid, ricinoleic acid, mixtures of these acids, etc. In place of the higher fatty acids, derivatives thereof such as glycerides and other esters may be employed. Actually we prefer to use glycerides of the fatty acids since products are obtained having superior softening properties to those resulting from the reaction of the polyamines with the free fatty acids. Products particularly suitable as textile lubricants and softeners are obtained by employing coconut oil to react with the polyamines in accordance with our invention since these products are dispersible in water without further solubilizing treatment and possess excellent lubricating and softening properties. As examples of other glycerides that may be employed in place of the long chain fatty acids there may be mentioned teaseed oil, castor oil, hydrogenated castor oil, etc.

The short chain acids employed in accordance with our invention contain from 2 to 5 carbon atoms; thus, for example, acetic acid, glycolic acid, lactic acid, glyceric acid, propionic acid, butyric acid and valeric acid may be employed; derivatives thereof such as esters, acid halides and anhydrides may be employed in accordance with procedures well known to the art. We prefer to use acetic acid or acetic anhydride in the preparation of our novel products because of their ready availability and the excellent softening properties of the amides prepared from these compounds.

In carrying out the reaction in accordance with our preferred method, approximately equimolecular quantities of a hydroxylated polyamine and a fatty acid containing from 8 to 22 carbon atoms are mixed; if a glyceride of a fatty acid is employed, e. g., coconut oil, approximately  $\frac{1}{3}$  mol of the glyceride per mol of polyamine is used. The compounds are then permitted to react at a temperature sufficiently high to cause the formation of the monoamide; this temperature may vary from about 120° C. to about 200° C., but preferably is between about 150° C. and about 170° C. The time for substantial completion of this reaction may vary widely depending somewhat upon the particular reactants and somewhat upon the temperature; generally, 8 hours or more are required. The pressure under which the reaction is carried out is preferably atmospheric; however, pressures above or below atmospheric may be employed. The product of the reaction is then mixed with a suitable quantity of a short chain fatty acid containing from 2 to 5 carbon atoms; as above mentioned, anhydrides, esters or acid halides of these acids may also be employed. The amount of short chain acid compound employed depends to some extent upon the number of amino groups to be acylated and the nature of the compound used. Thus, in the case of a triamine such as ethanol diethylene triamine, we prefer to employ about 1 mol of a short chain fatty acid per mol of triamine, leaving 1 amino group free for conversion to the salt; however, in the case of ethanol triethylene tetramine where it is desired to acylate all but one of the secondary amino groups, approximately 2 mols of the short chain acid per mol of the polyamine may be employed. It is to be understood that if derivatives of the short chain acid are reacted with the monoamide the amounts thereof will be adjusted accordingly; for example, approximately one-half mol of acetic

anhydride is used where one mol of acetic acid is required. If desired, sufficient amounts of the short chain acid may be used so that the —NH— group adjacent to the long chain fatty group may also be acylated. Generally, it may be said that the number of mols of short chain fatty acid employed per mol of polyamine will be equivalent to the number of groups to be acylated in accordance with our invention. The conditions under which this reaction is carried out may vary widely but we have found that the constituents may be reacted at atmospheric pressure and at a temperature of about 135° C. for about 3 to 5 hours, the mixture then raised to between about 150° C. and about 170° C. and the reaction continued for about 5 to about 8 additional hours with excellent results. However, it is to be understood that these conditions may be varied somewhat without affecting the course of the reaction, e. g., pressures above or below atmospheric may be used, the temperatures may vary widely so long as they are sufficiently high to effect acylation and the time of reaction may differ from the time above set forth.

The products of our invention may be liquids or solids, but generally they are solids. The majority of these products are relatively insoluble in water; however, products somewhat soluble or dispersible in water may be obtained. As above mentioned, the coconut oil products are generally dispersible in water. Certain products of our invention contain a free secondary amino group so that they may be treated with weak acids such as acetic acid or lactic acid to solubilize the amides and render them more soluble or dispersible in water. The solubilizing treatment is preferably carried out by mixing a dilute solution of the weak acid with the molten alkylol polyamide, stirring the mixture until it is homogeneous and permitting the mixture to cool. Our novel products may be marketed as such or in the form of an aqueous solution, dispersion or paste thereof. They may be applied to textile material by any of the well known methods, e. g., in the form of a dilute solution thereof, and in every case impart excellent softness, drape, flexibility and handle to the textile material.

The following examples are illustrative of our invention. Amounts are given in parts by weight:

#### EXAMPLE I

Coconut oil..... 679 parts (1 mol)  
Ethanol ethylene diamine..... 321 parts (3 mols)  
Acetic anhydride..... 181 parts (1½ mols)

The coconut oil and ethanol ethylene diamine were mixed in an open kettle and agitated at temperatures between 150° C. and 170° C. for 8 hours. The reaction product was then mixed with the acetic anhydride, the mixture agitated at a temperature of 135° C. for 5 hours, the temperature then raised to between 150° C. and 170° C. and the reaction continued for 5 more hours. The product was a clear, reddish amber liquid dispersible in water. The resultant product was highly suitable as a textile lubricant and softener.

#### EXAMPLE II

Hydrogenated soyabean oil..... 67.5 parts (1 mol)  
Ethanol ethylene diamine..... 23.0 parts (3 mols)  
Acetic acid (70%)..... 13.5 parts (3 mols)

The hydrogenated soyabean oil and ethanol ethylene diamine were heated together at temperatures in the range 140°-150° C. for 6 hours. The acetic acid was then added to the reaction mix-

ture and the temperature was raised to 175° C. and held at this temperature for 2 hours. Water was evolved during this latter portion of the reaction. The reaction mixture, when cool, was a solid condensation product of light brown color. The product was soluble in water and was suitable for use as an emulsifying and dispersing agent, particularly in the preparation of textile water-proofing compositions.

10

Stearic acid..... 284 parts (1 mol)  
Ethanol ethylene diamine..... 104 parts (1 mol)  
Acetic anhydride..... 51 parts (½ mol)

15 The foregoing reactants were condensed together in the same manner as were the corresponding ingredients in Example I. The resultant condensation product was a solid soluble in dilute acid solutions.

20

Oleic acid..... 282 parts (1 mol)  
Ethanol ethylene diamine..... 104 parts (1 mol)  
Acetic anhydride..... 51 parts (½ mol)

25 The above ingredients were reacted together exactly as were the corresponding ingredients of Example I. The resultant composition was readily dispersible in aqueous solutions.

30

EXAMPLE V

Refined corn oil..... 65.5 parts (1 mol)  
Ethanol ethylene diamine..... 23.2 parts (3 mols)  
Acetic anhydride..... 11.3 parts (1½ mols)

35 The corn oil and ethanol ethylene diamine were heated together in a closed kettle at temperatures in the range of 125-135° C. for 8 hours. At this time an alkali determination conducted upon a sample of the reaction mixture showed 12% of alkalinity in the mass, calculated as ethanol ethylene diamine, indicating that approximately one-half of the amino alkalinity had been blanked off by amidification. The mixture was then cooled to 70° C. and the acetic anhydride slowly added.

40 45 The temperature was then raised to 165° C. and maintained for a further 5 hours. At the end of this time the acid number of reaction mass was 10. The reaction mixture, when cooled, consisted of a brown colored liquid which was dispersible in water and was capable of producing water-in-oil emulsions.

50

EXAMPLE VI

Lauric acid chloride..... 40 parts (1 mol)  
Ethanol ethylene diamine..... 17.5 parts (1 mol)  
Glyceric acid..... 12 parts (1 mol)

55 The lauric acid chloride and ethanol ethylene diamine were agitated together at 170° C. for 7 hours. The resultant product was cooled to 70° C., the glyceric acid was added and the reaction was resumed at 170° C. and continued for 5 additional hours. The resultant condensation product was clearly soluble in water and exhibited excellent lubricating properties.

60

Oleic acid..... 282 parts (1 mol)  
Ethanol ethylene diamine..... 104 parts (1 mol)  
Glycollic acid (70% aqueous)..... 106 parts (1 mol)

65 70 The oleic acid and ethanol ethylene diamine were agitated together at temperatures between 150° and 170° C. for 10 hours and thereafter the mixture was cooled to 120° C. and the glycollic acid added. The reaction was resumed and continued

at 150° C. for 3 hours. The resultant amide condensation product had outstanding fiber lubricating properties.

## EXAMPLE VIII

|                         |                    |
|-------------------------|--------------------|
| 1,3 diamino isopropanol | 90 parts (1 mol)   |
| Stearic acid            | 284 parts (1 mol)  |
| Acetic anhydride        | 51 parts (1/2 mol) |

The 1,3 diamino isopropanol and stearic acid were heated together at temperatures ranging 175°-200° C. for 10 hours. Thereafter the mixture was cooled to 70° C., the acetic anhydride added and the temperature again raised to 200° C. for an additional 4 hours.

## EXAMPLE IX

## Textile treatment

Cotton sheeting was passed through a quench containing a 1/4% aqueous dispersion of the condensation product of Example I. A smooth, soft and even handle resulted on the dried fabric.

## EXAMPLE X

|                                                         | Parts |
|---------------------------------------------------------|-------|
| Paraffin wax (melting point 127° F.)                    | 21    |
| Condensation product produced in accordance with Ex. II | 2     |
| Basic aluminum acetate                                  | 3     |
| Water                                                   | 74    |
|                                                         | 100   |

The paraffin wax and condensation product were melted together and a solution prepared from the water and aluminum acetate was gradually introduced into the melt with agitation. The resultant emulsion constituted a stable stock emulsion from which more dilute solutions could be prepared for application to textiles for waterproofing preparations. For example, a 2% solution was applied to cotton fabric and the fabric was dried. A highly satisfactory waterproofing effect was developed upon the fabric.

## EXAMPLE XI

## Water-in-oil emulsion

|                                     | Parts |
|-------------------------------------|-------|
| Mineral seal oil                    | 22.5  |
| Condensation product of Example III | 2.5   |
| Water                               | 75.0  |
|                                     | 100.0 |

The condensation product and mineral seal oil were dissolved at 45° C. and thereafter the water was heated to 45° C. and slowly introduced into the melt with steady agitation. The result was a water-in-oil (as distinguished from an oil-in-water) emulsion which was suitable for many purposes, for instance, as a base for agricultural sprays, as a lubricant in the molding of ceramic materials, as a defoamer, and for many other purposes.

## EXAMPLE XII

## Paper tissue softening

A 1% solution of the hydroxy acetic acid salt of the condensation product produced in accordance with Example IV was sprayed onto a tissue paper during the manufacture thereof just prior to its entry into the calender stack. The paper so produced was softened and flexibilized in a very satisfactory manner.

## EXAMPLE XIII

## Fat liquor

|                                                                                                | Parts |
|------------------------------------------------------------------------------------------------|-------|
| Neat's-foot oil                                                                                | 3     |
| Hydroxy acetic acid solution of the condensation product produced in accordance with Example V | 5     |
| Water                                                                                          | 92    |
|                                                                                                | 100   |

The foregoing constituents were emulsified together and formed a highly satisfactory fat liquor which was used in lubricating alum tanned kid leather. The leather so treated was characterized by highly satisfactory softness and flexibility.

From the foregoing discussion and examples it will be seen that this invention provides novel and excellent polyamide textile lubricants and softeners. The polyamides of this invention impart to the textile material treated therewith a high degree of softness, drape, flexibility and handle, but do not cause any appreciable yellowing of the material even after prolonged contact therewith. The products of our invention have been found to give a softer finish when applied to textiles than the fatty amides of unsymmetrical dialkyl diamines hereinabove referred to; hence, smaller amounts of our products may be used to soften textiles than are necessary when the latter amides are employed. Furthermore, our products cause less discoloration of the textile material to which they are applied than do the amides of unsymmetrical dialkyl diamines. In addition, the products of our invention are much easier to use than the amides of the unsymmetrical dialkyl diamines since they may be dispersed or dissolved in water with great ease in contrast to the difficulties encountered in dispersing or dissolving the latter amides. As above pointed out, our novel products may be prepared from readily available and inexpensive amines and hence are much cheaper than the fatty amides of the unsymmetrical dialkyl diamines. Therefore, in view of the above, it is evident that the products of this invention display a marked superiority over lubricants and softeners heretofore used in the textile industry and hence will be of great value to textile manufacturers.

In addition to their use as textile lubricants and softeners, the products of this invention may be employed for a wide variety of other purposes; for example, they may be used as lubricants and softeners for fibrous materials generally such as leather, paper, etc. They may also be added to viscose spinning baths to prevent clogging of the spinnerettes and may be used as defoaming agents, assistants in dyeing, printing and otherwise treating textiles and the like, and for the preparation of detergents, and wetting, dispersing and emulsifying agents.

Having described our invention, what we claim as new and desire to secure by Letters Patent is:

1. A hydroxylated polyamide having the formula:



wherein  $R_1 - CO -$  represents a fatty acyl radicle containing from 8 to 22 carbon atoms;  $- OC - R_2$  represents a fatty acyl radicle containing from 2 to 5 carbon atoms;  $Z$  represents an aliphatic linking radicle having an unsatisfied valence at

both ends thereof chosen from the class consisting of (a) aliphatic hydrocarbon radicles, (b) aliphatic hydrocarbon radicles having a hydrogen atom replaced by a hydroxyl group and (c) aliphatic hydrocarbon radicles and aliphatic hydrocarbon radicles having a hydrogen atom replaced by a hydroxyl group which radicles are interrupted by groups selected from the class consisting of imino and neutralized imino groups;  $R_3$  in each occurrence, and independently of its other occurrence, represents a substituent chosen from the class consisting of hydrogen atoms, alkyl groups, aliphatic acyl groups and alkylol groups; with the proviso that at least one of the substituents  $R_3$  and  $Z$  must contain a hydroxyl group.

2. Alkylol polyamides having the general formula:



wherein  $R_1-CO-$  represents a fatty acyl radicle containing from 8 to 22 carbon atoms;  $-OC-R_2$  represents a fatty acyl radicle containing from 2 to 5 carbon atoms;  $R_3$  in each occurrence, and independently of any other occurrence, represents a substituent chosen from the group consisting of hydrogen, alkyl groups, aliphatic acyl groups and alkylol groups, with the proviso that at least one of the  $R_3$  substituents must be an alkylol group;  $R_4$  in each occurrence, and independently of any other occurrence, represents a substituent chosen from the group consisting of hydrogen and alkyl groups; and  $n$  represents a small whole number from one to three, inclusive.

3. Alkylol polyamides having the general formula:



wherein  $R_1-CO-$  represents a fatty acyl radicle containing from 12 to 18 carbon atoms;  $-OC-R_2$  represents a fatty acyl radicle containing from 2 to 5 carbon atoms;  $R_3$  in each occurrence, and independently of any other occurrence, represents a substituent chosen from the group consisting of hydrogen, alkyl groups, aliphatic acyl groups and alkylol groups, with the proviso that at least one of the  $R_3$  substituents must be an alkylol group;  $R_4$  in each occurrence, and independently of any other occurrence, represents a substituent chosen from the group consisting of hydrogen and alkyl groups; and  $n$  represents a small whole number from one to three, inclusive.

4. Alkylol polyamides having the general formula:



wherein  $R_1-CO-$  represents the fatty acyl radicles contained in a fatty glyceride oil;  $-OC-R_2$  represents a fatty acyl radicle containing from 2 to 5 carbon atoms;  $R_3$  in each occurrence, and independently of any other occurrence, represents a substituent chosen from the group consisting of hydrogen, alkyl groups, aliphatic acyl groups and alkylol groups, with the proviso that at least one of the  $R_3$  substituents must be an alkylol group;  $R_4$  in each occurrence, and independently of any other occurrence, represents a substituent chosen from the group consisting of hydrogen and alkyl groups; and  $n$  rep-

resents a small whole number from one to three, inclusive.

5. Alkylol polyamides having the general formula:



wherein  $R_1-CO-$  represents a fatty acyl radicle containing from 8 to 22 carbon atoms;  $-OC-R_2$  represents a fatty acyl radicle containing from 2 to 5 carbon atoms;  $R_3$  in each occurrence, and independently of any other occurrence, represents a substituent chosen from the group consisting of hydrogen atoms, alkyl groups, aliphatic acyl groups and alkylol groups, with the proviso that at least one  $R_3$  substituent must be an alkylol group; and  $n$  represents a small whole number from one to three, inclusive.

6. Alkylol diamides having the general formula:



wherein  $R_1-CO-$  represents a fatty acyl radicle containing from 8 to 22 carbon atoms;  $-CO-R_2$  represents a fatty acyl radicle containing from 2 to 5 carbon atoms; and  $R_3$  in each occurrence, and independently of its other occurrence, represents a substituent selected from the group consisting of hydrogen atoms, alkyl groups, aliphatic acyl groups and alkylol groups, with the proviso that at least one of the  $R_3$  substituents must be an alkylol group.

7. A diamide having the formula:



wherein  $R_1-CO$  represents the fatty acyl radicles contained in coconut oil.

8. A polyamide having the formula:



wherein  $R_1-CO$  represents the fatty acyl radicles contained in hydrogenated soyabean oil.

9. A polyamide having the formula:



wherein  $R_1-CO$  represents the fatty acyl radicles of corn oil.

10. Process for the preparation of polyamides which comprises amidifying an alkylol polyamine by heating at a temperature between about 120° C. and about 200° C. with approximately an acid molecular equivalent of a compound selected from the group consisting of fatty acids containing from 8 to 22 carbon atoms and the esters thereof, and with an amount of a compound selected from the group consisting of fatty acids containing from 2 to 5 carbon atoms, and the esters, an-

hydrides and acid halides thereof sufficient to react with the number of amino groups to be amidified therewith.

11. Process for the preparation of polyamides which comprises amidifying an alkylol polyamine by heating at a temperature between about 120° C. and about 200° C. with approximately a third of a molecular equivalent of coconut oil, and with an amount of a compound selected from the group consisting of fatty acids containing from 2 to 5 carbon atoms, and the esters, anhydrides and acid halides thereof sufficient to react with the number of amino groups to be amidified therewith.

EDWIN A. ROBINSON. 15  
MAURICE J. KELLEY.

## REFERENCES CITED

The following references are of record in the file of this patent:

## UNITED STATES PATENTS

|    | Number    | Name            | Date          |
|----|-----------|-----------------|---------------|
| 5  | 2,090,595 | Jacobson        | Aug. 17, 1937 |
|    | 2,139,679 | Hardy           | Dec. 13, 1938 |
| 10 | 2,279,497 | Sallmann et al. | Apr. 14, 1942 |
|    | 2,321,186 | Christmann      | June 8, 1943  |
|    | 2,243,329 | De Groote       | May 27, 1941  |
|    | 2,243,980 | Rheiner et al.  | June 3, 1941  |
|    | 2,345,632 | Robinson et al. | Apr. 4, 1944  |